

Feb. 8, 1944.

N. A. ZIEGLER ET AL

2,340,854

MALLEABLE CAST IRON

Filed Nov. 5, 1942

Fig. 1.



SILICON ADDITION TO EACH HEAT--  
0.5%

LEAD ADDITIONS:-

HEATS: 2491-0.01%

2494-0.03%

2495-0.04%

2496-0.05%

A.S.T.M. SPECIFICATION  
MINIMUM FOR ELONGATION

AFTER ANNEALING 52 HOURS

AFTER ANNEALING 17 HOURS

Fig 2.



YIELD POINT  
(UPPER POINT REPRESENTS  
TENSILE STRENGTH)

A.S.T.M. SPECIFICATION  
MINIMUM FOR TENSILE STRENGTH

A.S.T.M. SPECIFICATION  
MINIMUM FOR YIELD POINT

Inventors:  
Nicholas A. Ziegler,  
Homer W. Northrup

By: Joseph O. Lange, M.M.

## UNITED STATES PATENT OFFICE

2,340,854

## MALLEABLE CAST IRON

Nicholas A. Ziegler, Chicago, Ill., and Homer W. Northrup, Chattanooga, Tenn., assignors to Crane Co., Chicago, Ill., a corporation of Illinois

Application November 5, 1942, Serial No. 464,684

4 Claims. (Cl. 148—21.8)

This invention relates to improvements in metals and more particularly to a group of alloys suitable for making better malleable iron castings. The latter after being subjected to a suitable malleableizing heat treatment will possess improved tensile strength and yield point in accordance with the highest commercial standards, and with ductility, expressed in terms of percentage elongation, superior to that found in conventional material not treated in accordance with our invention.

At the outset, it should be understood that malleable iron is first produced as a white iron with practically all of its carbon in the combined form. It is subsequently rendered soft and ductile by means of annealing for prolonged periods at temperatures customarily in the range of 1560 to 1850° F. thereby causing the undissolved combined carbon or iron carbide to change to graphite; then follows cooling to a temperature in the vicinity of the critical range. The final product sought is a microstructure consisting of rounded particles of temper carbon (graphite) embedded in a soft iron matrix.

The present invention contemplates the production of a high-quality malleable cast iron by the addition of small amounts of lead, the purpose of such addition being to obstruct the formation of flake graphite in the white iron, and also in combination therewith by employing an annealing cycle less time-consuming than the prior-art processes.

It is well known to those skilled in the art that silicon (as well as other "graphite formers" like copper or nickel) promotes the formation of graphite. This is equally true regarding the formation of (1) flake graphite during the solidification period, resulting in a product known as "gray iron," and (2) temper carbon during the "annealing" or "malleableizing" of originally white iron, resulting in the product known as "malleable iron." It is equally well accepted that manganese (as well as other "carbide formers" such as chromium, molybdenum, tungsten, and the like) acts in exactly opposite direction, i. e. the formation of graphite is retarded and the formation of "combined carbon" or carbide is promoted.

In the art of manufacturing malleable castings it thus becomes necessary to balance silicon and manganese so that upon solidification no free or flake graphite would be formed and all carbon

would be present in combined form as carbides. At the same time these carbides should be sufficiently unstable so that upon reheating to the malleableizing temperatures they would break up or graphitize into temper carbon in reasonably short time periods. Thus it is always desirable to have in the malleable iron as much silicon as is permissible without developing flake graphite in the original (white) castings during the solidification period. It has been shown by various investigators that silicon greatly accelerates the malleableizing process (the formation of temper carbon) by increasing the number of temper-graphite particles per unit volume, thereby reducing the distance the carbon has to diffuse before precipitating as graphite. It also has been shown that the malleableizing rate is accelerated not only by the ease of graphite nucleus formation and the mobility of the carbon atom, but is also influenced by the relative stability of the original combined carbon (carbides). In other words, it is desirable to add to the molten white iron some element which would stabilize and promote the formation of combined carbon (carbides) upon solidification, but, at the same time, during the malleableizing heat treatment, would not interfere with (and preferably would promote) the breaking up of these carbides and formation of temper carbon.

We have discovered that by the introduction of up to 1.0% of lead into the molten metal, the formation of temper carbon is facilitated, or, in other words, the tendency of the iron to solidify white is enhanced.

Lead is cheaper than many of the prior elements used as a "whitener" such as tellurium, for example, and may therefore be used in much larger quantities at the same or, perhaps, even lower cost.

The experimental irons investigated were all made of standard cupola malleable scrap.

Fig. 1 shows comparative elongation test results.

Fig. 2 shows comparative tensile strength and yield point test results.

In the first of our series of tests 0.5% silicon was melted with the charge in an amount which would inoculate the metal and cause it to turn to the gray state. Then each heat was treated with a different amount of lead, ranging from 0.01% (heat 2491) to 0.2% (heat 2498).

Table 1

| Heat No.  | Lead            | Appearance of fractures          |                        |
|-----------|-----------------|----------------------------------|------------------------|
|           |                 | Fracture bar 1.5 in. diam.       | Test bar 0.5 in. diam. |
| 2491..... | Percent<br>0.01 | 0.75" gray center, white<br>rim. | Slightly mottled.      |
| 2494..... | 0.03            | .....do.....                     | Do.                    |
| 2495..... | 0.04            | 1/4" gray center, white rim.     | All white.             |
| 2496..... | 0.05            | 0.75" gray center, white<br>rim. | Slightly mottled.      |
| 2497..... | 0.10            | Slightly mottled.....            | All white.             |
| 2498..... | 0.20            | All white.....                   |                        |

A study of the appearances of fractures of the fracture bars and of the test bars as shown in Table 1 indicates that with progressively larger amounts of lead added, the fractures become more and more white until, with the addition of 0.2% lead, mottling completely disappears. The iron resulting from the treatment of our invention preferably has the following typical analysis:

|                 |               |
|-----------------|---------------|
| Silicon.....    | .5 to 2.5%    |
| Manganese.....  | .3 to 1.0%    |
| Sulphur.....    | .2% maximum   |
| Phosphorus..... | .4% maximum   |
| Carbon.....     | 1.5 to 3.5%   |
| Lead.....       | Trace to 1.0% |
| Iron.....       | The remainder |

In the accompanying drawing Fig. 1 shows a superposed chart arrangement of the minimum specifications of the American Society for Testing Materials (A. S. T. M.) relative to elongation, while Fig. 2 shows the yield point and tensile strength in comparison with the physical properties of the novel composition of our invention based upon the tests referred to.

The charts comprising the drawing are graphic representations of the physical properties of test specimens presented in tabular form in Table 2.

Table 2

| Heat No.<br>(two tests<br>each: a and b) | Tensile strength<br>in lbs. per<br>sq. in. after<br>annealing time<br>of— |             | Yield point<br>in lbs. per<br>sq. in. after<br>annealing time<br>of— |             | Elongation in<br>percent after<br>annealing time of— |             |
|------------------------------------------|---------------------------------------------------------------------------|-------------|----------------------------------------------------------------------|-------------|------------------------------------------------------|-------------|
|                                          | 52<br>hours                                                               | 17<br>hours | 52<br>hours                                                          | 17<br>hours | 52<br>hours                                          | 17<br>hours |
|                                          |                                                                           |             |                                                                      |             |                                                      |             |
| 2491:<br>a.....                          | 42,100                                                                    | 41,800      | 31,100                                                               | 34,000      | 10.0                                                 | 6.5         |
| b.....                                   | 40,300                                                                    | 41,500      | 30,700                                                               | 34,500      | 9.0                                                  | 6.0         |
| 2494:<br>a.....                          | 42,300                                                                    | 43,800      | 32,200                                                               | 35,200      | 10.0                                                 | 8.0         |
| b.....                                   | 40,600                                                                    | 43,100      | 31,900                                                               | 34,600      | 7.5                                                  | 8.0         |
| 2495:<br>a.....                          | 42,500                                                                    | 41,700      | 33,400                                                               | 35,700      | 8.5                                                  | 6.0         |
| b.....                                   | 42,600                                                                    | 36,200      | 33,100                                                               | 32,800      | 10.5                                                 | 6.0         |
| 2496:<br>a.....                          | 42,250                                                                    | 45,900      | 34,500                                                               | 35,800      | 6.0                                                  | 5.5         |
| b.....                                   | 43,400                                                                    | 45,500      | 34,700                                                               | 34,000      | 7.5                                                  | 8.5         |

The physical properties obtained in the specimens resulted from annealing times of 52 and 17 hours respectively, both periods being substantially shorter than the time required in general foundry practice. The production of a high-quality malleable iron after a comparatively short-time annealing process is another indication of the favorable effect of our lead treatment.

It is well known that in malleable iron the desired ductility, expressed as elongation, is a more difficult property to develop than the tensile strength. The elongation percentages shown in Table 2 and represented graphically in Fig. 1 of the drawing indicate that the addition of lead (in the amounts specified in the space in the upper

right-hand corner of the drawing) result in a malleable iron casting possessing superior ductility.

In the cases described in the foregoing paragraphs, silicon was melted with the metal charge and lead was added before pouring, but while the crucible was still in the furnace and the molten bath in a state of agitation. In the following experiments the heats were treated to imitate ladle additions, i. e. the crucible was taken out of the furnace and just before pouring, received first silicon, then a lead addition. Heats identified by the numbers 2520, 2521 and 2522 were treated in this way. The results are tabulated in Table 3.

Table 3

| Heat No.  | Lead            | Appearance of fractures    |                        |
|-----------|-----------------|----------------------------|------------------------|
|           |                 | Fracture bar 1.5 in. diam. | Test bar 0.5 in. diam. |
| 2520..... | Per cent<br>0.5 | Very slightly mottled..... | Very slightly mottled. |
| 2521..... | 0.75            | Slightly mottled.....      | White.                 |
| 2522..... | 0.75            | .....do.....               | Do.                    |

It may therefore be concluded from the test results presented that a malleable iron of the conventional composition, when treated with small amounts of lead (up to 1.0%) will possess desirable physical properties and a white fracture appearance, after annealing for a period of time substantially shorter than that required in general foundry practice.

While we have described our invention by referring to certain practical embodiments in order that a clear disclosure may be made to those skilled in the art, it will be understood that the scope of our invention is of broad application and not to be limited except as may be determined by the following claims read in light of the prior art.

We claim:

1. A white cast iron comprising the following elements as essential constituents in approximately the proportions given: silicon 0.5-2.5%, manganese 0.3-1.0%, sulphur 0.2% maximum, phosphorus 0.4% maximum, carbon 1.5-3.5%, to which is added lead in amounts from a trace up to 1.0%, the remainder being iron.

2. A white cast iron to be malleableized comprising the following elements as essential constituents in approximately the proportions given: silicon 0.5-2.5%, manganese 0.3-1.0%, sulphur 0.2% maximum, phosphorus 0.4% maximum, carbon 1.5-3.5%, to which is added lead in amounts from a trace up to 1.0%, the remainder being iron.

3. The process of making a malleable cast iron article comprising casting a mixture containing 1.5-3.5% carbon, 0.5-2.5% silicon and not less than about 94% iron, in the presence of a small but effective amount of lead, up to 1.0% of the mixture, the content of the latter element being sufficient to obstruct the formation of carbon in flake form during solidification, thereby producing a white cast iron article and then annealing the article under conditions to cause separation of at least a portion of the carbon as temper carbon.

4. As an article of manufacture, a malleableized cast iron having temper carbon and containing 1.5 to 3.5% carbon, a graphitizing agent equivalent in effect to 0.5 to 2.5% silicon and lead in small but effective amounts not to exceed 1.0%.

NICHOLAS A. ZIEGLER.  
HOMER W. NORTHRUP.